

[54] COMPOSITION OF BATHS AND ADDITIVES  
FOR ELECTRODEPOSITION OF BRIGHT  
ZINC FROM AQUEOUS, ALKALINE,  
ELECTROPLATING BATHS

[75] Inventors: William E. Rosenberg, Parma;  
Herbert H. Geduld, University  
Heights, both of Ohio

[73] Assignee: R. O. Hull & Company, Inc.,  
Cleveland, Ohio

[22] Filed: July 27, 1972

[21] Appl. No.: 275,534

**Related U.S. Application Data**

[63] Continuation-in-part of Ser. No. 116,649, Feb. 18,  
1971, abandoned.

[52] U.S. Cl. .... 204/55 Y, 204/DIG. 2, 204/55 R

[51] Int. Cl. .... C23b 5/10, C23b 5/46

[58] Field of Search..... 204/55 R, 55 Y, 432, 44

[56]

**References Cited**

**UNITED STATES PATENTS**

|           |        |              |            |
|-----------|--------|--------------|------------|
| 2,791,554 | 5/1957 | Winters..... | 204/55 Y   |
| 3,227,638 | 1/1966 | Burnson..... | 204/55 Y X |
| 3,655,534 | 4/1972 | Kampe.....   | 204/55 R   |

Primary Examiner—G. L. Kaplan

Attorney, Agent, or Firm—Watts, Hoffman, Fisher & Heinke

[57]

**ABSTRACT**

It has been found that the addition of the reaction product of a 1-halo-2, 3-epoxypropane and an amine selected from the group consisting of secondary and tertiary cycloaliphatic amines to aqueous, alkaline electroplating baths containing zinc ions, provides smooth, bright deposits of zinc.

4 Claims, No Drawings

**COMPOSITION OF BATHS AND ADDITIVES FOR ELECTRODEPOSITION OF BRIGHT ZINC FROM AQUEOUS, ALKALINE, ELECTROPLATING BATHS**

**CROSS-REFERENCES TO RELATED APPLICATIONS**

This application is a continuation-in-part of our pending application Ser. No. 116,649, filed Feb. 18, 1971, now abandoned.

**BACKGROUND OF THE INVENTION**

This invention pertains to improvements in the electrodeposition of zinc from aqueous, alkaline plating baths.

The electroplating of bright zinc coatings from aqueous, alkaline baths containing 7.5 to 150 gms. of sodium cyanide per liter is commonly achieved at present through the use of many widely known addition agents. However, the removal of the poisonous cyanide from the rinse water and sewage as required by law and health regulations can be carried out only at a very great expense, and the required safety measures render zinc plating by means of cyanide containing baths so expensive that in many cases it can no longer be carried out economically.

The widely known addition agents that provide bright deposits of zinc from alkaline, cyanide containing plating baths have little or no effect in the cyanide-free, alkaline baths. The deposits obtained in this case are dark, and spongy above a current density of 10 amps. per square foot. With this invention, bright electrodeposits can be obtained at a current density range of from 0 to over 150 amps per square foot, with or without the use of sodium cyanide. This wide current density range and elimination of the need for poisonous cyanide in the bath provides a novel, practical method of producing bright electrodeposits of zinc.

**SUMMARY OF THE INVENTION**

The present invention comprises an aqueous, alkaline electroplating bath, for producing a bright, lustrous, electrodeposit of zinc, containing zinc ions, and dissolved therein at a concentration of about 0.01 to about 10 gms. per liter, the reaction product of a 1-halo-2, 3-epoxypropane and a substance selected from the group consisting of secondary and tertiary cycloaliphatic amines, of the following general formulae:



where  $n$  is 1 to about 2,000,  $\text{R}_1$  is hydrogen or hydroxymethyl and  $\text{R}_2$  is hydrogen, hydroxy or piperazino.

The invention is also an aqueous addition agent for aqueous alkaline zinc electroplating baths, consisting essentially of from about 1:100 to 100:1 parts by weight of the reaction product of a 1-halo-2, 3-epoxypropane and a substance selected from the group consisting of secondary and tertiary cycloaliphatic amines of the above formulae.

**DETAILED DESCRIPTION**

The reaction products of a 1-halo-2, 3-epoxypropane and a substance selected from the group consisting of

secondary and tertiary cycloaliphatic amines of the following formulae:



where  $n$  is 1 to about 2,000,  $\text{R}_1$  is hydrogen or hydroxymethyl and  $\text{R}_2$  is hydrogen, hydroxy or piperazino are not at present available in commerce. However, all of the reactants are readily available or are easily synthesized and the reaction is easily accomplished with excellent reproducibility. The reactants that are not available in commerce are the cycloaliphatic amines where  $\text{R}_1$  and  $\text{R}_2$  are not hydrogen. These reactants are made by simply adding stoichiometric amounts of formaldehyde to solutions of piperazine at room temperature with mixing. The reactants are added to a vessel equipped with a reflux condenser and enough water to obtain one molar concentration. The reaction mixture is stirred vigorously and heated at reflux until a clear single phase is obtained. The mole-ratio of 1-halo-2, 3-epoxypropane to amine can vary from about 0.5/1 to about 2/1. The following examples will further demonstrate this preparation:

**EXAMPLE I**

60 gms. of N-methyl piperazine is added to a vessel containing 660 ml. of water. The solution is heated to 140°F., with stirring and 92 gms. of epichlorohydrin is added dropwise over a 35 minute period. Upon completion of the addition of epichlorohydrin, the mixture is heated to reflux and stirred for 1 hour. The solution is then allowed to cool, giving a clear, light yellow liquid of approximately 1 molar concentration.

The reaction products of this invention may be used in combination with any of the widely used brightening agents, e.g., gelatin, glue, peptone, anisaldehyde, piperonal, veratraldehyde, vanillin, 3-substituted-N-alkyl pyridinium halide, and quaternary aliphatic amines, said brightening agents being present in amounts from about 0.005 to about 5 gms. per liter. The brightening compositions of this invention are preferably used in the form of aqueous addition agents and contain from about 100:1 to about 1:100 parts by weight of the reaction product.

While the addition agents of this invention are effective in many aqueous, alkaline zinc plating bath formulations, it is preferred to use any of the basic baths described in the following examples. It will be understood that the following examples are just illustrations and are not meant to limit the use of the invention to these bath compositions only.

**EXAMPLE II**

| Bath Composition                                                                     | Concentration gms/liter |
|--------------------------------------------------------------------------------------|-------------------------|
| Zinc Oxide                                                                           | 9                       |
| Sodium Hydroxide                                                                     | 75                      |
| Reaction product of epichlorohydrin and N-methyl piperazine at 1 molar concentration | 5                       |

## EXAMPLE III

| Bath Composition                                                                     | Concentration gms/liter |
|--------------------------------------------------------------------------------------|-------------------------|
| Zinc Oxide                                                                           | 5                       |
| Sodium Hydroxide                                                                     | 75                      |
| Reaction product of N-Methyl Piperazine and epichlorohydrin at 1 molar concentration | 2                       |
| Veratraldehyde                                                                       | 0.1                     |

## EXAMPLE IV

| Bath Composition                                                                    | Concentration gms/liter |
|-------------------------------------------------------------------------------------|-------------------------|
| Zinc Oxide                                                                          | 9                       |
| Sodium Hydroxide                                                                    | 75                      |
| Reaction product of epibromohydrin and N-methyl piperazine at 1 molar concentration | 2                       |
|                                                                                     |                         |

## EXAMPLE V

| Bath Composition                                                                    | Concentration gms/liter |
|-------------------------------------------------------------------------------------|-------------------------|
| Zinc Oxide                                                                          | 9                       |
| Sodium Hydroxide                                                                    | 75                      |
| Reaction product of epibromohydrin and N-methyl piperazine at 1 molar concentration | 2                       |
| Anisaldehyde                                                                        | 0.1                     |

All testing was done in a conventional 267 ml. Hull Cell using steel panels and a zinc anode. Two ampere panels were run for 10 minutes at a temperature of 80°F. In every case the reaction product was compared to equal molar amounts of the reactants. In all tests the reaction products produced bright zinc deposits over a wide current density range, whereas the reactants produced only dull and coarse zinc deposits.

Having thus described this invention in such full, clear, concise and exact terms as to enable any person skilled in the art to which it pertains to make and use

the same, and having set forth the best mode contemplated of carrying out this invention, we state that the subject matter which we regard as being our invention is particularly pointed out and distinctly claimed in what is claimed, it being understood that equivalents or modifications of, or substitutions for, parts of the above specifically described embodiment of the invention may be made without departing from the scope of the invention as set forth in what is claimed.

10. What is claimed is:

1. An aqueous, alkaline, electroplating bath for producing a bright, lustrous electrodeposit of zinc, containing zinc ions, and dissolved therein about 0.01 to about 10 gms. per liter of a reaction product obtained by the reaction of a 1-halo-2, 3-epoxypropane and an amine at about a 0.5/1 to about 2/1 mole ratio of halo epoxypropane to amine, the amine being selected from the group consisting of secondary and tertiary cycloaliphatic amines of the following general formula:



25. where  $n$  is about 1 to about 2,000,  $\text{R}_1$  is hydrogen or hydroxymethyl, and  $\text{R}_2$  is hydrogen, hydroxy or piperazine, at a reaction temperature of about 140°F. to reflux for about 1 hour and a sufficient amount of water to give about a 1 molar solution.

30. 2. A bath composition as set forth in claim 1 wherein there is also dissolved up to about 150 gms. of sodium cyanide per liter.

35. 3. A bath composition as set forth in claim 1 wherein the 1-halo-2, 3-epoxypropane is epichlorohydrin.

40. 4. The plating bath composition as set forth in claim 1 wherein there is also present at least one of the substances selected from the group consisting of gelatin, glue, peptone, anisaldehyde, piperonal, veratraldehyde, vanillin, a 3 substituted -N-alkyl pyridinium halide and a quaternary aliphatic amine and present in a concentration of about 0.005 to about 5 gms. per liter.

\* \* \* \* \*